

June 30, 1925.

1,543,833

G. EGLOFF ET AL

TREATED CARBONACEOUS FUEL

Filed Feb. 10, 1921



Witnesses,  
John B. Mann

Inventors,  
Gustav Egloff,  
Harry P. Benner  
By Frank L. Belknap. 1714

Patented June 30, 1925.

1,543,833

# UNITED STATES PATENT OFFICE.

GUSTAV EGLOFF AND HARRY P. BENNER, OF INDEPENDENCE, KANSAS, ASSIGNEES  
TO UNIVERSAL OIL PRODUCTS COMPANY, OF CHICAGO, ILLINOIS, A CORPORATION  
OF SOUTH DAKOTA.

## TREATED CARBONACEOUS FUEL.

Application filed February 10, 1921. Serial No. 443,745.

*To all whom it may concern:*

Be it known that we, GUSTAV EGLOFF and HARRY P. BENNER, both citizens of the United States, residing in the town of Independence, county of Montgomery, and State of Kansas, have invented certain new and useful Improvements in Treated Carbonaceous Fuel, of which the following is a specification.

10 This invention relates to improvements in carbonaceous fuel and refers more particularly to an oil saturated carbon produced by the cracking of heavy petroleum oils such as fuel oil, Mexican or California crudes, bottom settling or the like.

15 In the cracking of heavy fuel oils, much pitchy carbon is precipitated which is suitable for use as fuel. In the cracking of, for example, Wayside fuel oil, on a commercial scale in the manner hereinafter described, 6925 gallons of said fuel oil produced 2300 pounds of oil soaked pitchy carbon which can be used as a fuel, either for heating the cracking apparatus or boiler or for any 20 other useful fuel purposes. The production of this pitchy carbon is a large economical item in the cracking of heavy oils, such as asphaltic oils of high carbon forming properties.

25 As an illustration, a plant cracking 3000 barrels of fuel oil from the Kansas Wayside field would produce approximately 20 tons wet carbon a day. In cracking heavy crude petroleums such as heavy Mexican crude from the Panuco field, over 40 tons a day of wet carbon would be produced by the cracking of 3000 barrels a day. To illustrate the immensity of this carbon production, consider the following: The shipment of petroleum oil from the Panuco field was over a million barrels for the week ending August 28, 1920. If this amount of Panuco crude was cracked and it certainly will be desirable to crack it, there would be produced as 30 a maximum 17,000 tons of carbon per week. This carbon might be worth from \$5.00 to \$10.00 a ton. If desired, this wet carbonaceous fuel can be used in lump form either in the same manner by stoker or hand firing or it may be pulverized and used much the same as fuel oil with steam or a blower.

To more clearly illustrate the manner of producing this carbonaceous fuel, reference may be had to the accompanying drawing in

which the single figure represents a view 55 partly in side elevation and partly in vertical section of an apparatus in which the process may be carried out.

Referring in detail to the drawings, 1 designates the furnace having burner 2, 60 stack 3, and combustion chamber 4. In the combustion chamber is mounted the heating coil 5 which may, for example, be from 20 to 40 tubes, each 20 feet long, and connected in series. The inlet side of the coil or heating 65 element is connected to a feed pump 6 by charging line 7 having throttle valve 8. The raw fuel oil is fed to the coil through the pipe 9 having throttle valve 10 leading to any suitable source of supply. The discharge side of the coil is connected by transfer line 11 having throttle valve 12 to a vapor or expansion chamber 13. This expansion chamber 13 is of relatively large 70 size. A plurality of these expansion chambers may be used and so connected that one may be cut out to be cleaned and the other cut into the system to use. This is not shown for the reason that we are not here claiming the apparatus. Each expansion 75 chamber is provided with a residue drawoff pipe 14 having throttle valve 15 leading to any suitable storage receptacle. The member 13 is provided with a pressure gauge 16, vapor outlet pipe 17 having throttle valve 18 80 and leading to dephlegmator 19. The upper end of the dephlegmator is connected by vapor line 20 having throttle valve 21 to condenser coil 22 seated in condenser box 23. The lower end of the coil is connected by 85 pipe 24 through throttle valve 25 into receiver 26. This receiver 26 has a pressure gauge 27, liquid level gauge 28, liquid drawoff 90 29 having throttle valve 30 and gas outlet pipe 31 having throttle valve 32. 95

The process may be operated as follows: Fuel oil, as for example, from the Wayside field, having say, a Baumé gravity of 23 degrees, or Mexican or California crude oil of from 12 to 18 degrees Baumé gravity, 100 may be fed continuously through the heating coil, raised to a temperature of from 650 to 800 degrees F., and delivered in liquid phase to the expansion chamber or chambers. The whole system may be maintained under 105 a pressure of say, 100 to 150 pounds. Heavier vapors which enter the dephlegmator will be condensed and continuously

returned as reflux condensate to the system. In the apparatus of substantially the principle shown in the drawing, Wayside fuel oil was cracked and produced an amount 5 of wet pitchy carbon equal to that heretofore described.

As an essential feature of the present process, this wet pitchy carbon which may be continuously or intermittently drawn out of 10 the vapor chamber or other chambers where it collects is now treated so that it can be more readily shipped. This is effectively done by dissolving out the oily constituents by a solvent. A suitable solvent would be 15 the pressure distillate bottoms which would, of course, be available in a cracking process. The dissolving out of the oil of the liquid oily content would leave the pitchy material and carbon in such condition that it could be 20 pressed into briquettes for shipment.

As a modification of the process, it may be desirable at times to dissolve out both the liquid oil content and the pitchy material leaving a dry carbon which from certain oils 25 could be suitably used for metallurgical pur-

poses, electrodes, fillers for tires, tire casings and the like. In the carbon production from the cracking of such heavy carbon producing ends as Mexican crudes, briquettes may be the quickest and simplest way of 30 handling the carbon for shipment.

What is produced by the present process would be a dry carbon suitable for use as carbonaceous fuel and preferably produced as part of a continuous process or operation 35 of a cracking process.

We claim as our invention:

An artificial fuel composed of a residue obtained from the cracking of petroleum oil under heat and pressure, said fuel consisting 40 of a pitchy solid carbon which has been freed of its oily constituents and is in a substantially dry state, and obtained by subjecting the pitchy carbon residue to the action of pressure distillate produced by the 45 cracking of the petroleum oil to remove the liquid oil therefrom.

GUSTAV EGLOFF.  
HARRY P. BENNER.